

# UNITED STATES PATENT OFFICE.

ANGELO LUCERTINI, OF TERNI, ITALY.

## PROCESS OF PRODUCING ARMOR-PLATES FOR WARSHIPS AND OTHER STEEL ARTICLES WITHOUT CASE-HARDENING.

1,110,395.

Specification of Letters Patent. Patented Sept. 15, 1914.

No Drawing.

Application filed April 23, 1910. Serial No. 556,988.

To all whom it may concern:

Be it known that I, ANGELO LUCERTINI, a subject of the King of Italy, and residing at 2 Via Mazzini, Terni, Italy, have invented 5 certain new and useful Improvements in the Process of Producing Armor-Plates for Warships and other Steel Articles Without Case-Hardening, and of which the following is a specification.

10 This invention relates to processes for manufacturing armor plates and other steel articles of the type in which the plate or the like has imparted to it the necessary toughness and hardness without case hardening.

15 The object of the present invention is to provide an improved process of the above kind for manufacturing armor plates and the like.

The steel used in the present process contains iron, carbon, silicon, sulfur, phosphorus, manganese, chromium and nickel in such proportions that it is capable of being hardened without cementation.

20 It has been found that the best results are obtained with a steel containing the above-mentioned elements in the following proportions:—

|            |                       |
|------------|-----------------------|
| Carbon     | From 0.70 to 0.95 %   |
| Silicon    | From 0.100 to 0.200 % |
| Sulfur     | Not more than 0.03 %  |
| Phosphorus | Not more than 0.03 %  |
| Manganese  | From 0.20 to 0.30 %   |
| Chromium   | From 2.50 to 3.50 %   |
| Nickel     | From 3.0 to 4.0 %     |
| Iron       | From 90.99 to 95.50 % |

30 The preferred composition of the steel is as follows:—C=0.88%, Si=0.15%, S=0.03%, P=0.03%, Mn=0.26%, Cr=3.40%, Ni=3.80%, Fe=91.45%.

40 According to the character desired in the final product, and according to the requirements of the process the proportions of these constituents may be varied. For example, 45 in order to render the metal less resistant to the development of toughness and to prevent the development of brittleness, it is well to keep the proportions of sulfur, phosphorus and manganese as low as possible, the favorable influence of manganese not being necessary in the presence of high percentages of carbon and chromium. The percentages of nickel and chromium may also be modified, but not too widely, because otherwise in ad-

dition to the other drawbacks, the thermic treatment may be rendered more difficult.

The metal is cast in suitable molds of the usual type. It is preferable that the ingot when taken out of the mold should be allowed to cool gradually and uniformly to about 450°. The temperature of the ingot is then again raised to 750–850° C. whereupon it is slowly brought down to about 450° C. The temperature is then again raised to about 620° C. and kept thereat for some 65 hours. At this point before giving the ingot the proper temperature for rolling it is convenient to again lower the temperature to about 450° C.

70 Although this treatment has a useful influence and is sometimes indispensable, the ingot may also be treated according to the process generally used in the art provided the ingots are of a good metallic composition and not very large or they may also be 75 large if the rolling mill is a very powerful one. The ingot, as soon as it is removed from its mold, may therefore be transferred directly to the heating furnace of the rolling mill after lowering the temperature. 80

For rolling, the ingot is introduced into the heating furnace of the rolling mill, care being taken to avoid too great a difference of temperature between the ingot and the furnace and the heating is carried on uniformly 85 throughout the progress of the operation. The rolling is started at a temperature of about 1150° C. and carried out preferably in more than one heating, and in every case must be carried out in several passes. After 90 the rolling is finished and the plate is placed in the furnace for the thermic treatments, the temperature of the said furnace is slowly, gradually and uniformly lowered to about 400° C. and then again raised to a temperature of about 590–610° C. In carrying out 95 this treatment it is well to first adopt an annealing system which consists in annealing at two different temperatures, namely, a high temperature annealing at a temperature of about 750–900° C., and a low temperature annealing at about 590° to 630° C., the annealing at low temperature being followed by a tempering at low temperature. 100 After this the transformation of the granular into a fibrous structure is nearly finished. A piece of the armor plate can then be broken off in order that its fracture may be examined.

ined. If the result is not satisfactory it will be sufficient to repeat the tempering at a temperature of from 80-100° C., and occasionally it may be necessary to again anneal 5 the plate or to temper it at a high temperature. Before the plate is subjected to the next operation it is annealed at low temperature, (about 600° C.) followed by correcting in a press in order to remove irregularities 10 which may have been caused by the various manipulations to which the plate has been submitted.

The above described process, though there 15 is no case hardening, is rather long, but it is particularly suitable for the most unfavorable case of very thick armor plates in which the metallic composition is not too good.

The plate after the above described operations, is treated in suitable machines in order 20 to reduce it approximately to the dimensions and shape required, and is then planed and ground down to its proper thickness on the surface which for example is to form the outer skin of the ship.

25 The planing and grinding of the outer face of the plate in order to remove the decarburized surface is an operation of importance in the process. If, however, the percentage of carbon is very high, and the 30 heating for the rolling and forging operations or the thermic treatments, appears not to have too much decarburized the surface of the plate, the planing and grinding operations may also be omitted, and in this case a 35 careful hammering and cleaning of the surface will be sufficient. Thereupon the plate is bent in the press to its proper shape, after having been heated to a low temperature such as 600° C. or a little more, and if found 40 necessary this heating may be repeated.

If for special reasons of conformation, heating to a high temperature cannot be avoided, care should be taken that the temperature employed is not unnecessarily 45 high, the plate being then again subjected to annealing or tempering at a low temperature. If it is deemed necessary owing to the numerous heat treatments to which the plate may have been subjected after the planing 50 operation, the outer face of the plate may be protected with carburizing material such as soot, graphite or the like. The plate is then ready to receive the final treatment for differential tempering. This operation is 55 more difficult and requires greater care with a plate according to the present invention than is the case with plates reduced by the usual processes. The most important point is to render this operation much more rapid 60 than usual, with the object of obtaining a small depth of tempered zone, the heating being at a temperature of about 860° on the outer smooth surface to be hardened, and a temperature of about 600° C. or even less, 65 on the inner face.

The operation is more difficult for plates of small thickness. This difficulty can be overcome, however, by the following means:—(1) The use of a source of heat of a very high heating power. (2) The artificial increase of the thickness of the plate by interposing a metallic layer between it and the sand bed, and (3) Modifying the composition of the metal by lowering its percentage of nickel below the established 70 limit or even suppressing it altogether. The plate is then corrected in a press and submitted to finishing processes of known character. After the differential heating the plate is quenched.

Having now described my invention, what I claim as new and desire to secure by Letters Patent is:

1. A process for producing armor plates and other steel articles comprising the following steps: cooling and reheating the ingot preparatory to rolling, rolling the ingot, heating and cooling the rolled plate so as to transform the metal from a granular to a fibrous structure, reducing the plate approximately to the required shape and size, heating one side of the plate to a high temperature for hardening, and heating the other side to a low temperature for toughening and quenching the plate.

2. A process for producing armor plates and other steel articles comprising the following steps: cooling the ingot gradually and uniformly throughout its whole mass, heating the ingot to a high temperature and gradually cooling it, heating the ingot to a temperature which is lower than the before mentioned temperature and is maintained for some hours after which the ingot is heated and then rolled, heating and cooling the rolled plate so as to transform the metal from a granular to a fibrous structure, reducing the plate approximately to the required shape and size, heating one side of the plate to a high temperature for hardening and heating the other side to a low temperature for toughening, and quenching the plate.

3. A process for producing armor plates and other steel articles comprising the following steps: heating the ingot at a high temperature, heating the same at a low temperature, rolling the ingot, annealing the rolled plate at a high temperature, annealing the same at a low temperature, reducing the plate approximately to the required shape and size, heating one side of the plate to a high temperature for hardening and heating the other side to a low temperature for toughening.

4. A process for producing armor plates and other steel articles comprising the following steps: heating the ingot at a high temperature, heating the same at a low temperature, rolling the ingot, heating and

- cooling the rolled plate so as to transform the metal from a granular to a fibrous structure, reducing the plate approximately to the required shape and size, planing and 5 grinding the plate on one face, heating the face which has been planed and ground to a high temperature for hardening and heating the other side to a low temperature for toughening.
- 10 5. A process for producing armor plates and other steel articles comprising the following steps: taking an ingot of steel; heating to about 1150° C.; rolling the ingot in several passes; lowering the temperature of 15 the rolled plate to 400° C.; raising the temperature of the plate to about 590-610° C.; annealing the plate at about 600° C.; heating one side of the plate for hardening and the other side for developing toughness and 20 quenching the plate.
6. A process for producing armor plates and other steel articles comprising the following steps: taking an ingot of steel, heating the ingot to about 750-850° C., cooling 25 the ingot to about 450° C. heating the ingot to about 620° C. for some hours, cooling the ingot to about 450° C.; gradually heating the ingot to about 1150° C.; rolling the ingot in several passes; lowering the temperature 30 of the rolled plate to 400° C.; raising the temperature of the plate to about 590-610° C.; annealing the plate at about 600° C.; heating one side of the plate for hardening and the other side for developing toughness 35 and quenching the plate.
7. A process for producing armor plates and other steel articles comprising the following steps: taking an ingot of steel; heating to about 1150° C.; rolling the ingot in 40 several passes; lowering the temperature of the rolled plate to 400° C.; raising the temperature of the plate to about 590-610° C.; annealing the plate at a temperature of about 750-900° C.; annealing the plate at 45 a temperature of 590 to 630° C.; tempering the plate at a low temperature; annealing the plate at about 600° C.; heating one side

of the plate for hardening and the other side for developing toughness and quenching the plate.

8. A process for producing armor plates and other steel articles comprising the following steps: taking an ingot of steel, heating the ingot to about 750°-850° C., cooling the ingot to about 450° C., heating the 55 ingot to about 620° C. for some hours, cooling the ingot to about 450° C.; gradually heating the ingot to about 1150° C.; rolling the temperature of the rolled plate to 400° C.; 60 raising the temperature of the plate to about 590°-610° C.; annealing the plate at a temperature of about 750°-900° C.; annealing the plate at a temperature of 590°-630° C.; tempering the plate at a low temperature; 65 annealing the plate at about 600° C.; heating one side of the plate for hardening and the other side for developing toughness and quenching the plate.

9. A process for producing armor plates and other steel articles comprising the following steps: taking an ingot of steel; heating to about 1150° C.; rolling the ingot in several passes; lowering the temperature of the rolled plate to 400° C.; raising the temperature of the plate to about 590°-610° C.; annealing the plate at a temperature of about 750°-900° C.; annealing the plate at a temperature of 590° to 630° C.; tempering the plate at a low temperature; again tempering at a low temperature; annealing the plate at about 600° C.; correcting the plate in the press; reducing the plate to the desired form; heating the formed plate to at least 600° C.; heating one side of the plate 85 to 860° C. while maintaining the other at 600° C. and quenching the formed plate.

In testimony whereof I have affixed my signature in presence of two witnesses.

ANGELO LUCERTINI.

Witnesses:

DUILIO NARDONI,  
G. LENZI.